

## UNITED STATES PATENT OFFICE

2,287,153

## FOUNDRY FACING

Burgess P. Wallace, Brooklyn, N. Y.

No Drawing. Application May 11, 1940,  
Serial No. 334,613

3 Claims. (Cl. 22—180)

This invention relates to the casting of metals in ordinary sand molds and has for its particular objects the provision of a facing of the carbonaceous type which is peculiarly adapted to be suspended in water and delivered to the mold in the form of a spray, thus admitting of such facing being effectively applied as a substantial coating to all of the mold surfaces and particularly the vertical surfaces thereof with the result that the castings obtained in a subsequent casting operation are characterized by their smooth, fine, clean surfaces which are free from pits, pin holes, blow holes, as well as from burnt-in-sand or fused silica skins and from which castings the adhering sand is readily peeled, thus minimizing the brushing, tumbling or milling and pickling operations thereof. Further objects will hereinafter appear.

In the production of so-called pattern-true castings, it has been customary, heretofore, to employ facing materials such as graphite, for example to fill up or slick over the surface voids in the mold surface in such a manner as to avoid the sealing of such surfaces so as to prevent the escape of the steam and gases evolved from the molten metal when the same is poured thereinto, which facing serves as a refractory protective layer against the fusing or cutting action of the molten metal on the sand surface of the mold surface, thereby facilitating the peeling of the sand from the casting and thus minimizing the amount of brushing, tumbling or milling and pickling operations in order to remove extraneous silicious material from the surfaces of the casting. Such facing was usually either applied from a dust bag or by means of a so-called slicking operation wherein the facing was applied to the mold by means of a fine, soft, brush. However, when so applied, it has not been possible to effectively face the vertical surfaces of the sand mold and consequently in order to remove the burnt-in-sand or fused silica skins from such vertical surfaces, excessive brushing, tumbling, pickling and milling operations have been required. These operations were not only expensive and laborious but in many cases, because of the tendency to obliterate fine designs on the mold surfaces, they were decidedly objectionable.

My investigations have led to the discovery that it is possible to produce castings wherein all of the surfaces, including the vertical surfaces thereof, are pattern-true and essentially free from burnt-in-sand and difficult removable silica skins by applying the herein described facing composition to the mold surfaces in the form of

a spray. Furthermore, such improved product is peculiarly adapted for use in such spraying operations, since the same remains suspended in the liquid vehicle for relatively long periods of time, there being a minimum tendency for the same to settle out and thus it is possible to apply a substantially uniform layer of the facing to the vertical and other surfaces of the mold continually throughout the spraying operation and also all possibility of the nozzles becoming clogged during the spraying operations is avoided.

My improved carbonaceous facing is preferably prepared as follows:

15 A mixture of finely pulverized coke, karaya gum, dextrine and bentonite is introduced into a mixer equipped with suitable agitating devices and therein the same are intimately mixed together, the proportions thereof preferably comprising

|                               | Parts |
|-------------------------------|-------|
| Coke of say 200 mesh or finer | 200   |
| Karaya gum                    | 1.1   |
| Dextrine                      | 4.5   |
| 25 Bentonite                  | 9.0   |
| Total                         | 214.6 |

30 Preferably a very small percentage of a preservative such as one tenth of one per cent of either copper sulphate, beta naphthol, benzoate of soda or like common preservatives are added to the foregoing mixture to prevent fermentation of the gum and dextrine in storage.

35 In the application of the aforesaid facing composition to green sand molds, the same is intimately admixed with a relatively limited quantity of water, preferably about 5½ to 8 lbs. of the aforesaid facing product is admixed with 8 lbs. of water.

40 The aforesaid bentonite, as is well known, is a natural clay that contains a large percentage of aluminum hydrate and silicic acid (hydrated silica), together with impurities such as the oxides of iron, sodium and potassium. It has a high dye-adsorption test (see in this connection the paper entitled "Dye adsorption test" in the transactions of the American Foundry Men's Association for May 1923). For example, the 45 maximum dye-adsorption figure of ordinary clay is but about 12,000 whereas bentonite has a minimum dye-adsorption figure of about 25,000.

The aforesaid bentonite almost instantly gelatinizes when the facing product is admixed with 55 the water and thereby not only facilitates the

permanent suspension of the coke in the spray mixture but, as the water in the spray mixture gradually evaporates from the mold surface, the gelatinous bentonite serves to retain sufficient moisture to enhance the cementing action of the particles of the facing composition with the sand particles of the mold.

The karaya gum in the aforesaid facing product, while it does possess a material cementing action insofar as it tends to assist in binding the particles of the facing composition to the sand particles of the mold surface, yet primarily functions as a colloidal coke-suspending agent and materially assists the bentonite in that respect. However, of itself and without the presence of bentonite in the mixture, such gum is incapable of effecting as suitable a suspension of the facing composition in the water. The dextrine does not especially assist in effecting the suspensibility of the coke in the water of the spray mixture, but acts primarily as a cementing agent to cause the facing composition to adhere to the sand particles of the mold surface to which the spray mixture is applied.

My improved facing composition when admixed with water as aforesaid, may be stored for a week or two and still be susceptible of being stirred and forming a satisfactory mixture for spraying whereas if the coke alone were admixed with water in the same proportions but without there being any gum, any bentonite or dextrine present, the same would tend to settle to a hard residue if the mixture were allowed to stand overnight which could be stirred with great difficulty if at all.

The aforesaid facing composition, following its application to the mold, does not promptly dry to a dry skin but remains damp and for a considerable period of time thereafter will stick to the fingers if lightly touched.

In the event in the preparation of the facing composition it is desired to prevent any tendency of the bentonite to clump or cluster and thereby interfere with the uniform admixture of the bentonite with the coke, it is merely necessary to add sufficient water to the bentonite, before admixing the same with the coke, to form a thin slurry which latter is then admixed with the coke, gum and dextrine and then the resultant mixture is dried and comminuted.

The castings obtained from applying a spray such as herein described on the vertical or other surfaces of the mold, possess an even smoother surface than that obtained when a dry carbonaceous facing is applied to the mold surfaces from a dust bag because of the fact that the manner of application results in the facing composition being compacted under pressure in the cavities of the sand surface of the mold. Preferably, the air pressure employed to spraying the liquid composition onto a mold ranges from about 25 to 45 lbs. depending on the viscosity of the mixture.

While karaya gum is preferred as the gum ingredient of my improved facing composition because of its ability to absorb several times its bulk of water and form a gel, other gums having a somewhat similar property but to a lesser degree such as tragacanth gum, may be substituted therefor. Likewise, goulac, a by-product from the manufacture of sulphite paper pulp or molasses, or like products having generally similar adhesive qualities capable of cementing the carbonaceous particles of the facing to the

sand particles in the mold surface may be substituted for the dextrine.

The proportions of the gum, dextrine and bentonite with respect to the coke are not highly critical but may vary substantially, for example the amount of bentonite should not be sufficient to render the spray mixture too viscous to be free flowing through the spray nozzle and the amount of dextrine or its equivalent should preferably not be less than about 2 parts nor more than about 10 parts while the karaya gum or its equivalent should be present in an amount sufficient to materially assist in the suspension of the coke but not in a sufficient amount to render the spray mixture too viscous to be free-flowing so as to interfere with the application of the same as a spray to the mold surface.

The amount of water which is employed is preferably not more than twice the amount by weight of the amount of the facing composition and desirably the amount thereof is but some 50% to 60% greater than the amount of the facing composition. If too much water is added to the facing composition when preparing the spray mixture the facing applied to the mold surface will be too sloppy and consequently an insufficient amount of facing will adhere to the mold surface and furthermore, the same might tend to dislodge the sand particles of the mold surface and thereby prevent the production of a pattern-true casting.

My improved facing composition not only produces castings all of whose faces including the vertical walls are pattern-true and from which castings the adhering sand layer can be readily peeled but because of the characteristic properties of the water suspension of the facing composition, as hereinbefore set forth, the same is suitable for application in the form of a water spray to the sand surfaces of a mold with the consequence that the cost of application minimized and also the costs of finishing the casting are materially reduced as compared with castings prepared with other facing compositions.

The characteristic viscosity or stickiness of the karaya or equivalent gum, as well as its ability to swell and thicken the mixture, produces a suspension of the coke dust when the facing composition is admixed with water in the manner aforesaid, which cannot be accomplished with bentonite alone owing to the absence of such viscosity or stickiness characteristic in bentonite and as a consequence, my improved facing composition containing such a gum, remains in suspension for much longer periods of time and can, on settling, be far more easily re-suspended with slight stirring than is possible were bentonite alone employed as such suspending agent. However, such karaya gum alone even in the absence of any bentonite is capable of accomplishing the suspension of the coke dust if the proportions of such gum are substantially increased beyond that employed in the aforesaid example of my improved facing composition, nevertheless, the excessive amount of karaya gum required to effect such suspension imparts an objectionable viscosity or stickiness to the mixture which not only interferes with the proper spraying thereof but also materially increases the tendency of the spray mixture to clog the fine aperture in the spray nozzle employed to apply the same.

Applicant is well aware of the Patent No. 1,787,964 of Jan. 6, 1931, which discloses a facing containing coke, bentonite and dextrine and also

Patent No. 1,845,371 of Feb. 16, 1932, which discloses a facing composition wherein various gums are suggested as the equivalent of dextrine for the purposes of that patent and the claims of this application are therefore confined to the improvement on such compositions which is specifically set forth therein since neither of the foregoing patented compositions are susceptible of forming a water suspension possessing the characteristics of applicant's improved product as herein set forth.

Various modifications may be made in the hereindescribed facing composition without in any way departing from the spirit of my invention as embraced within the scope of the appended claims.

Having thus described my invention, what I claim and desire to obtain by United States Letters Patent is:

1. An intermediate product for use in a spray composition for metal casting sand molds comprising a dry mixture consisting principally of a carbonaceous dust, the particles of which are coated with an adhesive agent consisting of dextrine and are intimately admixed with at least 2% and not more than 10% of bentonite and said mixture containing not less than  $\frac{1}{4}\%$  and not exceeding 3% of a thickening agent belonging to the group consisting of karaya gum and tragacanth gum, said dry product being characterized by the fact that when admixed with one to two volumes by weight of water, then a water suspension of the composition can be obtained which is susceptible of being continually sprayed from a spray nozzle as a uniform coating upon the surface of a green sand mold and in

which suspension the composition remains suspended for long periods of time without the solids of the mixture becoming compacted in such a manner that they can not be readily re-suspended by merely manually stirring the mixture.

2. In a spray composition for metal-casting sand molds, comprising a water suspension containing at least 50% of water by volume and the solid content of which suspension contains a major percentage of coke dust, the particles of which are coated with an adhesive agent consisting of dextrine, also in excess of 2% and less than 10% of bentonite and from  $\frac{1}{4}\%$  and not exceeding 3% of a gummy thickening agent belonging to the group consisting of karaya gum and tragacanth gum and the said spray composition being highly stable, capable of remaining in prolonged suspension on standing and being especially adapted for application to a mold surface by spraying through a spray nozzle.

3. In a spray composition for metal-casting sand molds, comprising a water suspension containing at least 50% of water by volume and the solid content of which suspension contains at least 90% of coke dust, the particles of which are coated with an adhesive agent consisting of dextrine, also in excess of 2% and less than 10% of bentonite and from  $\frac{1}{4}\%$  and not exceeding 3% of a gummy thickening agent belonging to the group consisting of karaya gum and the said spray composition being highly stable, capable of remaining in prolonged suspension on standing and being especially adapted for application to a mold surface by spraying through a spray nozzle.

BURGESS P. WALLACE.